

June 23, 1964

B. L. CLARK

3,138,547

ELECTROSENSITIVE RECORDING SHEETS

Filed Oct. 23, 1959

FIG. 1



FIG. 2



INVENTOR  
BRYCE L. CLARK  
BY  
Carpenter, Abbott, Coulter & Kinney  
ATTORNEYS

## 1

3,138,547

ELECTROSENSITIVE RECORDING SHEETS  
Bryce L. Clark, St. Paul, Minn., assignor to Minnesota  
Mining and Manufacturing Company, St. Paul, Minn.,  
a corporation of Delaware  
Filed Oct. 23, 1959, Ser. No. 848,393  
23 Claims. (Cl. 204—2)

This invention relates to an electro-sensitive recording sheet. In one aspect this invention relates to an electro-sensitive recording paper for facsimile signals and the like.

Trends in modern technology have been placing increasing demands on fast, convenient and inexpensive techniques for printing line copy or continuous tone images and also for recording coded information. For example, recording information, such as speech and pictorial or scientific data from high speed aircraft or satellites in orbit, is assuming considerable significance. Also, high speed printing of the output of electronic computers is still seriously limited by the fact that the final recording stage is slow in comparison to the computation rate of the machine.

Various methods of recording by means of electric signals and various types of recording media have been known, but in general prior art methods and recording blanks employed therein have been subject to certain disadvantages. For example, it has been known to impregnate paper with electrically conductive solutions, or electrolytes, said solutions being adapted to be decomposed by signal impulses so that a record of the signals is made. It is also old to cause an electric arc to burn holes in a paper recording blank, the holes thus burned representing telegraphic signals for comprising the outlines of the subject matter desired to be recorded. Such recordings, however, are only suitable for relatively coarse work where no fine gradations of tonal values are necessary, such as in the reception of telegraphic signals in general and the recording of various types of curves in connection with process instrumentation. However, in the transmission of matter, particularly of pictures and the like, where continuous tones are encountered, the range of tonal values extends from what might be termed pure white to pure black, and the above methods have suffered from serious disadvantages, such as diffusion of the image area.

One of the most widely used types of electro-sensitive paper consists of a carbon impregnated conductive paper bearing, on one surface, a metallic paint layer and, on the other surface, a powdery light gray coating. During the recording process the light gray coating is at least partially displaced or removed by the passage of current from the stylus through the paper. Such sheets are difficult to handle because of the readily smeared, readily pressure marked surface. The current flow tends not only to alter the character of the light gray coating but also to disrupt the bonding or adhesion of the light gray masking coating to the adjacent carbon impregnated paper and to provide thereby a readily removable image.

Attempts have been made to produce dry electro-sensitive sheets which do not rely either on electrolytes or on the physical disruption of the sheet. Certain materials have been employed which decompose under the influence of heat generated by an electric current or which alter their form in an allotropic manner. However, in certain applications, as in various instruments measuring process variables, such sheets are subject to extremes of temperature, pressure, and the like. A satisfactory heat stable electro-sensitive sheet which is capable of producing a high contrast, well defined, smudge resistant, visible image which can potentially further be electronically scanned has not heretofore been known. It is therefore

## 2

an object of this invention to provide such an electro-sensitive paper with the above mentioned and other advantages.

It is an object of this invention to provide an electro-sensitive copysheet capable of reproducing smudge resistant, highly stable images with good definition and high contrast.

It is another object of this invention to provide an electro-sensitive sheet which is resistant to pressure marking, 10 mechanically strong and which is additionally capable of recording information which can be thereafter scanned and reproduced by electronic means.

An additional object of this invention is to produce an electro-sensitive facsimile sheet capable of reproducing an 15 image with substantially no dusting, flaking or smoking.

Another object of this invention is to provide a method for making an electro-sensitive paper with the above properties.

Still another object of this invention is to provide an 20 image bearing sheet which can be further developed by electrolytic means.

FIGURE 1 is a cross-sectional view of an electro-sensitive sheet according to this invention.

FIGURE 2 is a schematic diagram of a facsimile recording system embodying an electro-sensitive copysheet according to this invention.

The electro-sensitive sheets of this invention comprise a continuous electrically conductive layer and a contiguous layer comprising at least one water-insoluble, heat 30 stable, light insensitive, particulate metal compound capable of being electrically reduced in situ to the corresponding free metal, in a matrix of a binder having a lower electrical conductivity than said metal compound, said contiguous layer being essentially nondisplaceable 35 under the conditions of electrical reduction.

The electrically conductive layer may be any conductive material, including metal foil, paper or fabric impregnated with conductive particles, such as aluminum flakes, conductive glass, conductive plastics, etc. Flexible 40 sheets are generally used, particularly when the electro-sensitive sheet is wrapped around a rotatable roll or drum during the receipt of electrical facsimile signals and reproduction of the image. Although the nondisplaceable or nondisruptable nature of the contiguous layer or electro-sensitive topcoating permits the use of a carbon impregnated matrix, such as carbon impregnated paper, as the electrically conductive layer, this is not preferred because of other generally less desirable properties of carbon impregnated matrices, for example, relatively low tear strength, etc.

50 The electro-sensitive layer or topcoating contains a binder having a low electrical conductivity in which is uniformly distributed or dispersed at least one water-insoluble, heat stable, particulate metal compound which can be reduced to the corresponding free metal by the passage of electrical current, e.g. by means of a stylus. This current passage results in reduction of the particulate metal compound in the dry state. The free metal thereby produced in those areas contacted by a stylus provides a visible 55 reproduction of the electrical impulses or currents, the dark colored free metal varying in intensity with the current passed. In this manner, it is possible to produce varying tonal gradations in the image areas as the stylus scans the electro-sensitive layer with which it makes electrical contact.

60 Since it has now been found that a variety of diverse metallic compounds can be electrically reduced in this manner, selection depends on such factors as the color contrast desired, cost, toxicity, desired electrical requirements for reduction, etc. The following laboratory test procedure (Example 1) may be used to determine the 65 utility of a given metallic compound in the electro-sensitive sheets of this invention and will be used to define such 70

electrically reducible metal compounds within the scope of this invention.

#### EXAMPLE 1

To a wide mouth pint jar 80 grams of the particulate material to be evaluated is charged along with 20 grams of a 30:70 mol ratio copolymer of butadiene and styrene and 100 grams of toluene. One-half pint of 0.5 in. diameter glass or porcelain balls are added and the mixture is milled until an 8.5 or better fineness of grind, as measured on the Hegman fineness of grind gauge, is attained (usually about 8 hours of milling). With a 0.001" aluminum foil backing sheet positioned in a flat bed, notched bar knife coater, the knife was adjusted to provide a wet coating thickness of 3 mils. The above milled mixture is placed on the backing sheet behind the knife, and the backing sheet is thereafter pulled through the orifice to provide a uniform 3 mil thick wet coating. The coated sheet is thereafter allowed to dry at room temperature.

The dry coated sheet is then wrapped around a 3 inch diameter aluminum roll connected as anode to a variable D.C. source and is held securely in position by means of spring clips. A 10 mil diameter tungsten stylus, actuated by means of a screw drive lightly contacts the coated surface of the sheet and is moved progressively along an axis parallel to the axis of the metal roll. The stylus is connected as cathode to the variable D.C. source. Meters are provided to measure the voltage and current in the circuit. The metal roll is rotated at a peripheral speed of 100 inches/second and the stylus is advanced at a rate of 75 lines per inch. The voltage is slowly increased until a current flow is noted or to a maximum of 500 volts when no current flow is detected. When current flow is obtained, the voltage is held constant to observe the effect of the voltage and current on the coated sheet. The voltage is increased in increments with similar observation until an image or darkening of the surface under the stylus is observed. Those sheets on which are produced a dark image area in this manner are then analyzed to ascertain the presence of a free metal image. When no darkening is observed in this test procedure, the metal compounds are considered non-electrically reducible for purposes of this invention and can be employed as inert fillers. The following table illustrates the results obtained in this test using illustrative materials. This test can also be run with the stylus connected as anode and the aluminum roll connected as cathode. In ordinary facsimile machines, such as the Western Union "Intrafax" machine mentioned later, alternating currents are employed.

Table I.—Standard Image Formation Test

[4/1 Pliolite S-7 at 50% solids coated 3 mils wet on .001 aluminum foil]

| Particulate Material  |                        | Binder Material   |                                   | Sheet Color       | Image Conditions |               |              | Description                | Analysis |
|-----------------------|------------------------|-------------------|-----------------------------------|-------------------|------------------|---------------|--------------|----------------------------|----------|
| Name                  | Formula                | Name              | Description                       |                   | Formed           | Applied Volts | Current, ma. |                            |          |
| Zinc Oxide.....       | ZnO.....               | Pliolite S-7..... | 30:7 butadiene-styrene copolymer. | White.....        | Yes.....         | 100           | 10           | Black lines and holes..... | ZnO..... |
| Titanium Dioxide..... | TiO <sub>2</sub> ..... | do.....           | do.....                           | do.....           | No.....          | 500           | 0            | No evidence of image.....  |          |
| Lead Oxide.....       | PbO.....               | do.....           | do.....                           | Light yellow..... | Yes.....         | 450           | 2            | Black lines and holes..... | PbO..... |
| Magnesium Oxide.....  | MgO.....               | do.....           | do.....                           | White.....        | No.....          | 500           | 0            | No evidence of image.....  |          |

Inorganic, sulfur free metal compounds of a non-allotropic nature are preferred. Since these electrosensitive layers should be essentially uniform in electrical conductivity under a wide variety of environmental conditions, the materials incorporated therein preferably exclude light sensitive materials which darken on exposure to light or which vary substantially in conductivity in relation to the amount of impinging light. Moreover, as mentioned earlier, the electrosensitive sheets of this invention utilize an electrically reducible metal compound which is heat stable, i.e. which is not decomposed at sustained temper-

atures below about 200° C., preferably below about 250° C. Both organic and inorganic electrically reducible metal compounds are contemplated within the scope of this invention.

Visible image reproduction on the electrosensitive sheet is dependent on the contrast or color difference between the dark free metal containing image areas and the light unreduced background. Since a dark or white image is most desirable, the electrically reducible metal compound employed is preferably light in color, usually white or off-white. Such light colored metal compounds include, for example, zinc oxide, lead monoxide, basic lead carbonate, stannic oxide, barium sulfate, etc. However, electrically reducible metal compounds which are colored, such as vanadium pentoxide, silver oxide, cadmium sulfide, ceric oxide, zirconium oxide, antimony pentasulfide, cadmium oxide, etc., may be used in admixture with the lighter colored metal compounds or with light colored non-reducible pigments or fillers, such as titanium dioxide, magnesium oxide, etc. Of course, in certain applications, an immediately visible image is not necessary. The ratio of filler to the electrically reducible metal compound may be varied widely, depending on the desired definition, the desired color contrast and the resistivity required for efficient reduction of the electrically reducible metal compound in the electrosensitive layer.

The binder which is incorporated into the electrosensitive layer serves to firmly affix the particulate material onto the electrically conductive substrate and to maintain the continuity or integral nature of the layer. In the reproduction of images according to this invention, the current passing through the electrosensitive sheet tends to blast or disrupt the continuity of the particulate material if insufficient binder is employed. Thus, the particulate material to binder weight ratio is maintained below 10:1, preferably below 8:1 and above about 1:2. As mentioned earlier, the finely divided particulate material, i.e. the electrically reducible metal compound and filler, if used, is uniformly distributed throughout the binder matrix. Suitable insulating binders include various organic materials such as cellulose acetate, cellulose nitrate, ethyl cellulose, polystyrene, polyvinyl acetate, polyvinyl chloride, chlorinated rubbers, butadiene-styrene copolymer (e.g. 30:70 mol ratio), polyisobutylene, polymethacrylates, etc. Those particular electrically reducible metal compounds requiring a higher resistance of the electrosensitive layer to effect reduction to the free metal are preferably distributed in a matrix of those binders having higher resistance to electrical breakdown, since

decomposition of the binder is to be minimized and preferably precluded.

The resistance characteristics of the entire electrosensitive layer may be adjusted either by controlling the resistance or proportion of the binder and of the particulate material, or by controlling the thickness of the electrosensitive layer. It is also possible to control the resistance by controlling the fineness of the particulate particles. This resistance is regulated in such fashion as to impress sufficient electrical potential across said layer to effect efficient reduction of the metal compound in the

image areas and to permit reduction with essentially no disruption of the continuity of the electrosensitive layer. Inasmuch as the electrical resistance transversely through the electrosensitive layer is to be maintained at a substantially uniform value, with the variation in reduction being controlled by the intensities of the signaling currents or potentials, the layer thickness should be maintained at a substantially constant value throughout the useful area of the sheet. Layer thicknesses above about 0.5 mil, generally above about 1 mil, are usually employed. Ordinarily, the thickness need not exceed about 3 mils. The preparation of these electrosensitive layers with any particular electrically reducible metal compound or mixtures thereof by regulating the above factors to produce the optimum result will be readily apparent to persons skilled in the art.

When the electrosensitive sheets of this invention are used to reproduce an image transmitted by a facsimile process, as in FIGURE 2, the passage of electrical current from the scanning stylus (1), in contact with the electrosensitive surface of the copysheet (2), through the sheet to the metal drum (3) rotatable about axis (4), reduces the metallic compound in the image areas to a lower valence state, in which state the conductivity and other electrical properties of the image areas is sufficiently different from the equivalent properties of the background areas to afford a unique means not only for visual recording but also for the storage and reuse of

the recorded information. For example, the electrosensitive sheets of this invention can be provided in tape form and can be used to record information and data from electronic computers and the like. Such recorded information can then be reused both by optical or visual sensing means and potentially by electronic sensing means relying on the differential pattern of electrical properties. No satisfactory information storage sheets or tapes of this character have heretofore been found that possess this combination of potentially valuable properties.

Because of the differential conductivity pattern resulting from the production of a free metal containing image area, these electrosensitive sheets can be further processed to alter the character of the image. Electrolytic processes, in which the electrically conductive backing sheet is connected as the cathode and the electrosensitive layer is contacted by a suitable electrolyte, such as aqueous nickel chloride, an aqueous solution of a silver salt and thiourea, etc., can be used for further development of the image, if desired.

Using the preparative techniques described in Example 1, the electrosensitive sheets in Table II were prepared. Images were obtained by using these sheets on the standard Western Union "Intrifax" facsimile machine. The electrically conductive material of the backing was aluminum in all runs except for Example 28, in which a carbon impregnated paper (2000 ohms per square) was employed. All percents are percent by weight. P/B represents the weight ratio of particulate material to binder.

Table II

| Example | Partic./<br>Binder<br>Ratio | Particulate Materials                                              |         |                         |         | Binder Materials            |         | Coating<br>Wet<br>Mils | Sheet<br>Color | Image<br>Color | Image<br>Power |     |    |
|---------|-----------------------------|--------------------------------------------------------------------|---------|-------------------------|---------|-----------------------------|---------|------------------------|----------------|----------------|----------------|-----|----|
|         |                             | Name                                                               | Percent | Name                    | Percent | Name                        | Percent |                        |                |                | Volts          | Ma. |    |
| 2       | 4/1                         | TiO <sub>2</sub>                                                   | 48      | ZnO-HC4 <sup>1</sup>    | 32      | Pliolite S-7 <sup>2</sup>   | 20      | 3                      | White          | Black          | 105            | 32  |    |
| 3       | 4/1                         | ZnO-HC4                                                            | 80      |                         |         | do                          | 20      | 3                      | Light          | Dark           | 12             | 37  |    |
| 4       | 1/1                         | ZnO-HC4                                                            | 50      |                         |         | do                          | 50      | 3                      | gray           | gray           |                |     |    |
| 5       | 5/1                         | ZnO(USP) <sup>3</sup>                                              | 83.5    |                         |         | do                          | 16.5    | 3                      | White          | Black          | 80             | 12  |    |
| 6       | 8/1                         | ZnO(USP) <sup>3</sup>                                              | 88.8    |                         |         | do                          | 11.2    | 3                      | do             | Gray           | 75             | 30  |    |
| 7       | 6/1                         | ZnO(USP) <sup>3</sup>                                              | 85.7    |                         |         | Marbon HV 9200 <sup>4</sup> | 14.3    | 3                      | do             | Black          | 70             | 15  |    |
| 8       | 10/1                        | ZnO(USP) <sup>3</sup>                                              | 90.9    |                         |         | Saran F120 <sup>5</sup>     | 9.1     | 3                      | do             | Brown          | 105            | 30  |    |
| 9       | 5/1                         | ZnO(USP) <sup>3</sup>                                              | 83.5    |                         |         | Dow 700 <sup>6</sup>        | 16.5    | 3                      | do             | Black          | 60             | 10  |    |
| 10      | 6/1                         | ZnO(USP) <sup>3</sup>                                              | 85.7    |                         |         | Ethyl Cellulose Type N22    | 14.3    | 3                      | do             | do             | 45             | 20  |    |
| 11      | 10/1                        | ZnO(USP) <sup>3</sup>                                              | 90.9    |                         |         | Lucite 41 <sup>7</sup>      | 9.1     | 3                      | do             | Gray           | 40             | 22  |    |
| 12      | 6/1                         | ZnO(USP) <sup>3</sup>                                              | 85.7    |                         |         | Lemac 150 <sup>8</sup>      | 14.3    | 3                      | do             | Black          | 85             | 30  |    |
| 13      | 10/1                        | Ni <sub>2</sub> O <sub>3</sub>                                     | 90.9    |                         |         | Pliolite S-7                | 9.1     | 3                      | Dark           | do             | 155            | 50  |    |
| 14      | 4/1                         | CdO                                                                | 80      |                         |         | do                          | 20      | 3                      | Brown          | do             | 135            | 110 |    |
| 15      | 4/1                         | AgO                                                                | 80      |                         |         | do                          | 20      | 3                      | Black          | Gray           | 275            | 260 |    |
| 16      | 4/1                         | HgO                                                                | 80      |                         |         | do                          | 20      | 3                      | Orange         | Black          | 250            | 105 |    |
| 17      | 4/1                         | PbCO <sub>3</sub> (basic)                                          | 40      | ZnO-HC4                 | 40      | do                          | 20      | 3                      | Light          | do             | 65             | 42  |    |
| 18      | 4/1                         | BaSO <sub>4</sub>                                                  | 40      | ZnO-HC4                 | 40      | do                          | 20      | 3                      | do             | Brown          | 50             | 20  |    |
| 19      | 4/1                         | Bi <sub>2</sub> O <sub>3</sub>                                     | 40      | ZnO-HC4                 | 40      | do                          | 20      | 3                      | Yellow         | black          | 110            | 70  |    |
| 20      | 4/1                         | CeO                                                                | 60      | ZnO-HC4                 | 20      | do                          | 20      | 3                      | gray           | Tan            | 165            | 85  |    |
| 21      | 4/1                         | ZrO                                                                | 60      | ZnO-HC4                 | 20      | do                          | 20      | 3                      | Light          | Dark           | 285            | 190 |    |
| 22      | 5/1                         | ZnO(USP)                                                           | 66      | ZrO                     | 17      | do                          | 17      | 3                      | White          | Black          | 90             | 22  |    |
| 23      | 5/1                         | ZnO(USP)                                                           | 82.7    | HgO                     | 0.8     | do                          | 16.5    | 3                      | Buff           | do             | 85             | 17  |    |
| 24      | 5/1                         | ZnO(USP)                                                           | 82.7    | HgO                     | 0.8     | do                          | 16.5    | 3                      | do             | do             | 85             | 135 |    |
| 25      | 4/1                         | TiO <sub>2</sub>                                                   | 40      | {ZnO-HC18 <sup>9</sup>  | 12      | do                          | 20      | 3                      | White          | do             | 130            | 35  |    |
| 26      | 2/1                         | ZnO(XX602) <sup>10</sup>                                           | 50      | {ZnO(USP) <sup>11</sup> | 28      | }                           | do      | 33                     | 3              | Light          | Brown          | 105 | 40 |
| 27      | 4/1                         | PbO                                                                | 60      | ZnO-HC4                 | 17      | do                          | 33      | 3                      | gray           | black          | 175            | 100 |    |
| 28      | 5/1                         | ZnO(USP)                                                           | 82.7    | HgO                     | 0.8     | do                          | 16.5    | 3                      | Yellow         | Black          | 165            | 17  |    |
| 29      | 4/1                         | V <sub>2</sub> O <sub>5</sub>                                      | 80      | do                      | 20      | do                          | 20      | 3                      | do             | do             | 100            | 75  |    |
| 30      | 4/1                         | Sb <sub>2</sub> S <sub>3</sub>                                     | 60      | ZnO-HC4                 | 20      | do                          | 20      | 3                      | Orange         | Red            | 135            | 110 |    |
| 31      | 4/1                         | SnO <sub>2</sub>                                                   | 80      |                         |         | do                          | 20      | 3                      | Pale           | black          | 850            | 150 |    |
| 32      | 4/1                         | AgO <sub>2</sub> C(CH <sub>2</sub> ) <sub>20</sub> CH <sub>3</sub> | 80      |                         |         | do                          | 20      | 3                      | yellow         | do             | 135            | 13  |    |
| 33      | 4/1                         | ZnO(USP)                                                           | 63.2    | {PbO                    | 13.4    | do                          | 20      | 3                      | White          | do             | 135            | 40  |    |
| 34      | 2/1                         | ZnO(XX602)                                                         | 66      | {ZnO-HC4                | 13.4    | do                          | 20      | 3                      | Light          | Black          | 70             |     |    |
| 35      | 6/1                         | ZnO(USP)                                                           | 51.5    | {TiO <sub>2</sub>       | 25.7    | do                          | 17      | 3                      | gray           | do             | 80             | 30  |    |
| 36      | 6/1                         | H <sub>2</sub> MoO <sub>4</sub>                                    | 85.7    | {CdO                    | 8.5     | do                          | 17      | 3                      | Pink           | Black          | 70             | 17  |    |
| 37      | 4/1                         | Bi <sub>2</sub> O <sub>3</sub>                                     | 40      | ZnO-HC4                 | 40      | do                          | 20      | 1                      | Light          | Gray           | 220            | 10  |    |
| 38      | 4/1                         | Bi <sub>2</sub> O <sub>3</sub>                                     | 40      | ZnO-HC4                 | 40      | do                          | 20      | 2                      | gray           | Dark           | 60             | 45  |    |

See footnotes at end of table.

Table II—Continued

| Example | Partic./<br>Binder<br>Ratio | Particulate Materials                |         |                        |         | Binder Materials  |         | Coating<br>Wet<br>Mils | Sheet<br>Color     | Image<br>Color  | Image<br>Power |     |
|---------|-----------------------------|--------------------------------------|---------|------------------------|---------|-------------------|---------|------------------------|--------------------|-----------------|----------------|-----|
|         |                             | Name                                 | Percent | Name                   | Percent | Name              | Percent |                        |                    |                 | Volts          | Ma. |
| 39..... | 4/1                         | Bi <sub>2</sub> O <sub>3</sub> ..... | 40      | ZnO-HC4.....           | 40      | Pliolite S-7..... | 20      | 3                      | Light<br>yellow.   | Light<br>brown. | 90             | 50  |
| 40..... | 4/1                         | Bi <sub>2</sub> O <sub>3</sub> ..... | 40      | ZnO-HC4.....           | 40      | .....do.....      | 20      | 4                      | Gray<br>yellow.    | Dark<br>brown.  | 145            | 60  |
| 41..... | 4/1                         | Bi <sub>2</sub> O <sub>3</sub> ..... | 40      | ZnO-HC4.....           | 40      | .....do.....      | 20      | 5                      | Yellow             | Black.....      | 165            | 65  |
| 42..... | 2/1                         | ZnO(USP).....                        | 63.5    | Aluminum<br>flake..... | 3.5     | .....do.....      | 33      | 3                      | gray.<br>Gray..... | .....do.....    | 90             | 25  |

<sup>1</sup> ZnO-HC4 is high conductivity zinc oxide doped with free metal, supplied by New Jersey Zinc Company.

<sup>2</sup> Pliolite S-7 is 30:70 mole ratio butadiene-styrene copolymer supplied by Goodyear Tire & Rubber Co.

<sup>3</sup> ZnO (USP) is lead free, acicular French process zinc oxide supplied by New Jersey Zinc Co.

<sup>4</sup> Marbon HV9200 is a high viscosity chlorinated rubber supplied by Marbon Corp.

<sup>5</sup> Saran F120 is polyvinyl chloride resin supplied by Dow Chemical Co.

<sup>6</sup> Dow 700 is polystyrene resin supplied by Dow Chemical Co.

All of the image containing electrosensitive sheets of Table II were resistant to smudging and pressure marking.

Various other embodiments and modifications will become apparent to those skilled in the art from the above disclosure.

I claim:

1. An electrosensitive non-electrolytic recording sheet which comprises a continuous electrically conductive layer and a contiguous layer thereon comprising at least one water-insoluble, heat stable, light insensitive particulate metal compound capable of electrical reduction in situ to the corresponding free metal, said metal compound being uniformly dispersed in an inorganic matrix having a lower electrical conductivity than said metal compound, said contiguous layer being essentially non-displaceable under conditions required for said electrical reduction.

2. The electrosensitive sheet of claim 1 in which the weight ratio of particulate material to binder is below about 10:1.

3. The electrosensitive sheet of claim 1 in which the particulate metal compound is zinc oxide.

4. The electrosensitive sheet of claim 1 in which the particulate metal compound is nickel sesquioxide.

5. The electrosensitive sheet of claim 1 in which the particulate metal compound is cadmium oxide.

6. The electrosensitive sheet of claim 1 in which the particulate metal compound is silver oxide.

7. The electrosensitive sheet of claim 1 in which the particulate metal compound is basic lead carbonate.

8. The electrosensitive sheet of claim 1 in which the particulate metal compound is barium sulfate.

9. The electrosensitive sheet of claim 1 in which the particulate metal compound is bismuth trioxide.

10. The electrosensitive sheet of claim 1 in which the particulate metal compound is cerium oxide.

11. The electrosensitive sheet of claim 1 in which the particulate metal compound is zirconium oxide.

12. The electrosensitive sheet of claim 1 in which the particulate metal compound is lead oxide.

13. The electrosensitive sheet of claim 1 in which the particulate metal compound is vanadium pentoxide.

14. The electrosensitive sheet of claim 1 in which the particulate metal compound is antimony pentasulfide.

15. The electrosensitive sheet of claim 1 in which the particulate metal compound is stannic oxide.

<sup>7</sup> Lucite 41 is polymethylmethacrylate supplied by E. I. du Pont de Nemours and Co.

<sup>8</sup> Lemac 150 is polyvinyl acetate supplied by American Monomer Co.

<sup>9</sup> ZnO (XX602) is lead free, acicular American process zinc oxide supplied by New Jersey Zinc Co.

<sup>10</sup> Lucite 42 is polyethylmethacrylate supplied by E. I. du Pont de Nemours and Co.

<sup>11</sup> Dow V9 is polystyrene supplied by Dow Chemical Co. as a viscous, low viscosity liquid.

16. The electrosensitive sheet of claim 1 in which the particulate metal compound is silver behenate.

17. The electrosensitive sheet of claim 1 in which the particulate metal compound is molybdc acid.

18. The electrosensitive sheet of claim 1 in which the particulate metal compound is conductive zinc oxide.

19. An electrosensitive non-electrolytic recording sheet which comprises a non-carbonaceous electrically conductive layer and a contiguous layer thereon consisting essentially of at least one water-insoluble, heat stable, light insensitive particulate metal compound capable of electrical reduction in situ to the corresponding free metal, said metal compound being uniformly dispersed in an organic matrix having a lower electrical conductivity than said metal compound, said contiguous layer being essentially nondisplaceable under conditions required for said electrical reduction.

20. The electrosensitive recording sheet of claim 19 wherein said non-carbonaceous electrically conductive layer is a metal.

21. The electrosensitive recording sheet of claim 19 wherein said non-carbonaceous electrically conductive layer is aluminum.

22. The electrosensitive recording sheet of claim 19 wherein said non-carbonaceous electrically conductive layer is aluminum and said metal compound is conductive zinc oxide.

23. The electrosensitive recording sheet of claim 19 wherein said non-carbonaceous electrically conductive layer is aluminum, said metal compound is conductive zinc oxide, and said contiguous layer contains titanium dioxide filler.

#### References Cited in the file of this patent

#### UNITED STATES PATENTS

|           |        |               |
|-----------|--------|---------------|
| 2,281,013 | Talmy  | Apr. 28, 1942 |
| 2,319,765 | Talmy  | May 18, 1943  |
| 2,554,017 | Dalton | May 22, 1951  |

#### FOREIGN PATENTS

|         |               |               |
|---------|---------------|---------------|
| 149,268 | Switzerland   | Nov. 16, 1931 |
| 464,112 | Great Britain | Apr. 12, 1937 |
| 113,072 | Australia     | May 9, 1941   |
| 962,661 | Germany       | Apr. 25, 1957 |

UNITED STATES PATENT OFFICE  
CERTIFICATE OF CORRECTION

Patent No. 3,138,547

June 23, 1964

Bryce L. Clark

It is hereby certified that error appears in the above numbered patent requiring correction and that the said Letters Patent should read as corrected below.

Columns 3 and 4, Table I, under the heading "Analysis" the formula "ZnO" and "PbO" read -- Zn<sup>0</sup> --, and -- Pb<sup>0</sup> --; column 7, line 35, for "inorganic" read -- organic --.

Signed and sealed this 24th day of November 1964.

(SEAL)

Attest:

ERNEST W. SWIDER  
Attesting Officer

EDWARD J. BRENNER  
Commissioner of Patents